

# United States Patent [19]

Koch et al.

[11] 4,053,491

[45] Oct. 11, 1977

[54] BRANCHED-CHAIN ALIPHATIC ESTER OILS

[75] Inventors: Karlheinz Koch, Haan, Rhineland; Hermann Kroke, Erkrath-Unterbach, both of Germany

[73] Assignee: Henkel Kommanditgesellschaft auf Aktien, Dusseldorf, Germany

[21] Appl. No.: 602,825

[22] Filed: Aug. 7, 1975

Related U.S. Application Data

[63] Continuation-in-part of Ser. No. 428,887, Dec. 27, 1973, abandoned.

[30] Foreign Application Priority Data

Jan. 22, 1973 Germany ..... 2302918

[51] Int. Cl.<sup>2</sup> ..... C09F 5/08; C10M 1/24

[52] U.S. Cl. ..... 260/410.6; 252/56 S

[58] Field of Search ..... 260/410.6; 252/56 S

[56]

References Cited

U.S. PATENT DOCUMENTS

|           |         |               |          |
|-----------|---------|---------------|----------|
| 3,282,971 | 11/1966 | Metro .....   | 252/56 S |
| 3,341,574 | 9/1967  | Taylor .....  | 252/56 S |
| 3,441,600 | 4/1969  | Chao .....    | 252/56 S |
| 3,778,454 | 12/1973 | Kleiman ..... | 252/56 S |

FOREIGN PATENT DOCUMENTS

1,180,386 2/1970 United Kingdom ..... 252/56 S

Primary Examiner—Patrick P. Garvin

Assistant Examiner—John F. Niebling

Attorney, Agent, or Firm—Hammond & Littell

[57]

ABSTRACT

Branched-chain aliphatic ester oils comprising full esters of branched-chain aliphatic polyols having from 2 to 6 hydroxyl groups with saturated, branched-chain, aliphatic monocarboxylic acids having from 14 to 22 carbon atoms, as well as their use alone, or as mixture components, as lubricants or hydraulic fluids.

10 Claims, No Drawings

## BRANCHED-CHAIN ALIPHATIC ESTER OILS

## REFERENCE TO A PRIOR APPLICATION

This application is a continuation-in-part of our co-pending U.S. Patent application Ser. No. 428,887, filed Dec. 27, 1973, and now abandoned.

## THE PRIOR ART

So-called ester oils have found in the last few years a wide field of application as valuable lubricants. Thus, for example, for the lubrication of turbine engines of jet-propelled aircraft, esters of dicarboxylic acids and alcohols with medium chain length, such as, for example, dioctyl sebacate, or esters of various polyols with fatty acids with a medium chain length are used. More recently, such ester oils have also been used to an increased extent for other lubrication problems where the lubricating requirements are high, as for example, as mixing components in partly synthetic engine oils. The special suitability of the ester oils for these purposes is based on the facts that, compared with the usual lubricants based on mineral oil, they have a far more favorable behavior of viscosity with temperature and that, compared with substances of comparable viscosities, the pour point is distinctly lower. These properties also represent an essential requirement for the suitability of an oil as the operating fluid in hydraulic systems, since its viscosity is only allowed to alter to an insignificant extent with considerable temperature variations and besides it must also remain capable of use at low temperatures.

It is common knowledge to the technician that ester oils of higher viscosity usually prove less satisfactory in their behavior in the cold, since the increase of the viscosity generally accompanies an increase of the pour point. For lubrication problems which absolutely necessitate the use of more highly viscous ester oils, so-called complex esters have been recently developed. These contain as esterification components both diols or polyols and dicarboxylic acids in addition to monofunctional alcohols or acids, in order to be able to prepare esters with low acid and hydroxyl numbers. The viscosities of such complex esters at 100° F is about 30 to 300 cSt and is 210° F at 10 to 30 cSt. The pour points of such highly viscous complex esters do not generally lie below -30° C. Therefore, they are not satisfactory in this respect for many purposes of use. A further serious disadvantage of these complex esters is that their preparation causes great difficulties, since during the esterification of polyfunctional acids with polyfunctional alcohols, undesired polymerizations must be contemplated and controlled, if possible. The acid fractions or fractions of partial esters remaining in the complex ester after the esterification reaction can only be removed with difficulty by refining or distillation.

It has also already been attempted to prepare more highly viscous ester oils by esterification of polyfunctional alcohols with straight-chain monocarboxylic acids. If, however, the preparation of esters with high viscosities comparable with those possessed by the complex esters is desired, products are obtained of which the pour points rise to values above 0° C. As may be seen from the following Table I, a viscosity of over 30 cSt at 100° F with a trimethylolpropane ester can be obtained when an addition of fatty acids of chain lengths over C<sub>10</sub> is made as the esterification component. If, for example, lauric acid is used as esterification

component, a trimethylolpropane ester with a viscosity of 36.4 cSt at 100° F is obtained, but with a pour point of +7° C. The corresponding lauric acid-neopentylglycol ester has already a pour point of +11° C with a viscosity of only 16.2 cSt at 100° F.

TABLE I

| Ester                     | Pour Point in °C | Viscosity in cSt at 100° F | Viscosity Index |
|---------------------------|------------------|----------------------------|-----------------|
| <u>Trimethylolpropane</u> |                  |                            |                 |
| n-C <sub>8</sub> -acid    | -60              | 12.1                       | 113             |
| n-C <sub>9</sub> -acid    | -60              | 14.6                       | 128             |
| n-C <sub>10</sub> -acid   | -54              | 18.8                       | 138             |
| n-C <sub>11</sub> -acid   | -51              | 22.4                       | 143             |
| n-C <sub>12</sub> -acid   | -29              | 26.2                       | 145             |
| n-C <sub>12</sub> -acid   | +7               | 36.4                       | 143             |
| <u>Neopentylglycol</u>    |                  |                            |                 |
| n-C <sub>8</sub> -acid    | -62              | 5.95                       | 116             |
| n-C <sub>9</sub> -acid    | -27              | 9.18                       | 113             |
| n-C <sub>10</sub> -acid   | -27              | 11.3                       | 145             |
| n-C <sub>12</sub> -acid   | +11              | 16.2                       | 167             |

Further, the preparation of ester oils based on polyols and branched-chain fatty acids of medium chain length has already been attempted. When these fatty acids or mixtures of branched-chain and straight-chain fatty acids of medium chain length are used, the pour point of the esters obtained is indeed distinctly lower, but this advantage is offset by disadvantages in the behavior of the viscosity with temperature, as product result with a low viscosity index, as may be seen from the following collected results of Table II.

TABLE II

| Ester                     | Pour Point in °C | Viscosity in cSt at 100° F | Viscosity in cSt at 210° F | Viscosity Index |
|---------------------------|------------------|----------------------------|----------------------------|-----------------|
| <u>Trimethylolpropane</u> |                  |                            |                            |                 |
| n-C <sub>8</sub> -acid    | -54              | 19.0                       | 4.09                       | 138             |
| i-C <sub>8</sub> -acid    | -54              | 27.1                       | 4.72                       | 85              |
| mix-C <sub>8</sub> -acid  | -62              | 19.1                       | 3.92                       | 115             |
| <u>Pentaerythritol</u>    |                  |                            |                            |                 |
| n-C <sub>8</sub> -acid    | +1               | 34.7                       | 6.23                       | 135             |
| i-C <sub>8</sub> -acid    | -34              | 129.2                      | 11.60                      | 82              |
| mix-C <sub>8</sub> -acid  | -60              | 47.3                       | 7.07                       | 116             |

## OBJECTS OF THE INVENTION

An object of the present invention is the development of ester oils which, besides a very low pour point, have in comparison a high thermal stability, a high viscosity, and are at the same time satisfactory in their viscosity temperature behavior.

Another object of the invention is the development of a branched-chain aliphatic ester oil consisting essentially of a full ester of a branched-chain aliphatic polyol having from 2 to 6 primary hydroxyl groups selected from the group consisting of alkanepolyols having from 3 to 6 carbon atoms and alkoxyalkanepolyols having from 6 to 12 carbon atoms with  $\alpha$ -branched-chain alkanoic acids having the formula



wherein R<sub>1</sub> and R<sub>2</sub> are alkyl having from 1 to 19 carbon atoms and the total number of carbon atoms in the acid is from 14 to 22.

A further object of the invention is the development of lubricating and hydraulic fluid compositions contain-

ing from 20% to 100% of at least one of the above branched-chain aliphatic ester oils.

A yet further object of the present invention is the improvement in the method of facilitating the motion of one solid over the surface of another solid by interspersing a thin film of a lubricant between the surfaces of said solids in frictional contact which consists of employing the above branched-chain aliphatic ester oils as said lubricant.

These and other objects of the invention will become 10 more apparent as the description thereof proceeds.

### DESCRIPTION OF THE INVENTION

It has now been found that ester oils consisting of the full esters of

- a. branched, aliphatic polyols having 2 to 6 primary hydroxyl groups, and
- b. saturated,  $\alpha$ -branched-chain, aliphatic monocarboxylic acids with a total of 14 to 22 carbon atoms in the molecule satisfy the necessary requirements of a very 20 low pour point, a high thermal stability, a high viscosity and a satisfactory viscosity-temperature behavior to an extent not previously attained.

More particularly, the ester oil of the invention is a branched-chain aliphatic ester oil consisting essentially of a full ester of a branched-chain aliphatic polyol having from 2 to 6 primary hydroxyl groups selected from the group consisting of alkanepolyols having from 3 to 6 carbon atoms and alkoxyalkanepolyols having from 6 to 12 carbon atoms with  $\alpha$ -branched-chain alcanoic acids having the formula



wherein  $R_1$  and  $R_2$  are alkyl having from 1 to 19 carbon atoms and the total number of carbon atoms in the acid is from 14 to 22.

As the alcoholic component, all branched-chain aliphatic polyols having 2 to 6 primary hydroxyl groups form the basis of the ester oils according to the invention, such as the alkanepolyols having from 3 to 6 carbon atoms and the alkoxyalkanepolyols having from 6 to 12 carbon atoms, as for example, neopentylglycol, trimethylolpropane, pentaerythritol, or dipentaerythritol. The polyols neopentylglycol, trimethylolpropane and pentaerythritol are of particular importance.

Suitable acid components of the ester oils according to the invention are all saturated,  $\alpha$ -branched-chain, aliphatic monocarboxylic acids with a total of 14 to 22 carbon atoms in the molecule. More particularly, these acids are  $\alpha$ -branched-chain alcanoic acids having the formula



wherein  $R_1$  and  $R_2$  are alkyl having from 1 to 19 carbon atoms and the total number of carbon atoms in the acid is from 14 to 22. Such carboxylic acids are obtainable in various ways, as for example, by oxidation of the  $\alpha$ -branched-chain alcohols with a corresponding number of carbon atoms obtained from shorter chain alcohols by the Guerbet process. Another source of such carboxylic acids is provided by various  $\alpha$ -branched alcohols from petroleum chemistry, as well as the reaction products of conjugated diolefines, such as isoprene, pentadi-

ene-1,3, butadiene-1,3, etc. with methacrylic acid esters in the presence of an organometal complex of zero valent nickel and an electron donor according to German Patent (DOS) No. 2,025,830 and the commonly-assigned U.S. Patent appln. Ser. No. 146,780, filed May 25, 1971 now U.S. Pat. No. 3,855,255.

Of the  $\alpha$ -branched-chain carboxylic acids having a total of 14 to 22 carbon atoms in the molecule obtainable in the above-mentioned and other ways, special importance is attached to those saturated, branched-chain carboxylic acids in which the chain branches in the  $\alpha$ -position to the carboxyl group and the two alkyls of the chain branches are straight-chained. The preparation of such saturated,  $\alpha$ -branched-chain carboxylic acids may be effected, for example, by the Guerbet reaction on unbranched saturated alcohols of medium chain length to give alcohols of the desired total number of carbon atoms, branched in the 2 position, which are subsequently oxidized to give a carboxyl group in place of the alcohol group. Another method, for example, is the hydrogenation of the  $C_{20}$  carboxylic acid obtained by the reaction of 1,3-butadiene with methyl methacrylate in the presence of an organometal complex of zero valent nickel and an electron-donor and subsequent saponification, according to the German Patent Specification (DOS) No. 2,025,830. The unsaturated ester is likewise described in U.S. Pat. No. 3,660,440. A nonadecanecarboxylic acid obtained in this way has, for example, the structure  $[CH_3(CH_2)_8]_2 = CH - COOH$ .

Other carboxylic acids branched in the  $\alpha$ -position to the carboxyl group can also be obtained by oxidation of branched-chain alcohols from petroleum chemistry, as for example, by the oxidation of an isomeric mixture of branched-chain  $C_{16}$  alcohols of the structure



which can be prepared by aldol condensation of isoctylaldehyde, which itself is obtainable from isoheptene, which is formed during the cracking of petroleum. The two  $C_6H_{13}$ - and  $C_8H_{17}$ -groups of the carboxylic acids branched in the  $\alpha$ -position so obtained are themselves also branched.

Particularly favorable results can be obtained with saturated, branched-chain, aliphatic monocarboxylic acids in which the chain is branched in the  $\alpha$ -position to the carboxyl group, the branches are themselves straight-chain, and the total number of carbon atoms in the molecule of which is 16. Of the  $C_{16}$ -carboxylic acids branched in the  $\alpha$ -position to the carboxyl group, isopalmitic acid obtained by oxidation of 2-hexyl-decanol formed from n-octanol in the Guerbet synthesis is of very special importance. The ester oils obtained by use of this isopalmitic acid show extremely favorable properties with respect to stability at high temperatures and behavior in the cold as well as of its viscosity behaviors.

The esters according to the invention consisting of branched, aliphatic polyols having 2 to 6 primary hydroxyl groups and the saturated,  $\alpha$ -branched-chain, aliphatic monocarboxylic acids with a total of 14 to 22 carbon atoms, can be prepared by the usual esterification processes, such as by heating the reactants in the presence of an esterification catalyst, as for example, tin or aluminum powder, or p-toluenesulfonic acid and

other substances. In the preparation of the isopalmitic acid ester it has proved satisfactory to free the ester obtained from acid residues by washing with a short-chain alcohol, such as methanol. Obviously the purification of the crude reaction mixture from excess acid can also be carried out by washing with caustic alkali liquors.

The ester oils according to the invention are outstandingly suitable both alone, and in admixture with other products already known for this purpose, for use as lubricants and as hydraulic fluid, on account of their extremely favorable properties with regard to viscosity, behavior in the cold and thermo-stability. Such a favorable overall behavior cannot be obtained with all previously known ester oils obtainable in such a simple manner. Owing to their relatively high viscosity and their favorable viscosity behavior with temperature, the ester oils according to the invention can be used advantageously also in those fields which have previously been barred to the complex esters. When used as a mixture component in lubricants and hydraulic fluids, any desired mixing proportions can be selected, which are determined exclusively by the values required with respect to working behavior, pour point and viscosity-temperature behavior. In general, however, the total product does not contain a fraction less than 20%. Both mineral oils and other ester oils are suitable as mixing components, depending on the purpose of use. These compositions contain from 20% to 100% of the ester oils of the invention.

The following Examples further describe the invention without it being restricted thereto.

### EXAMPLES

The full esters of the invention utilized for testing for behavior to cold and viscosity-temperature behavior were prepared from the polyols and branched-chain carboxylic acids as given below by the method outlined above of heating an excess of about 1.2 mol of acid for each mol equivalent of hydroxyl groups in the polyol in the presence of a p-toluenesulfonic acid to a temperature of about 125° C while removing the water produced by the reaction. The esters were recovered by washing the reaction mixture with methanol.

A = Neopentylglycol

B = Trimethylolpropane

C = pentaerythritol

D = Isopalmitic acid, obtained by oxidation of the 2-hexyl-decanol formed from n-octanol by oxidation in the Guerbet synthesis

E = Nonadecanecarboxylic acid of the structure



The values obtained during the tests are given in the following Table III.

TABLE III

| Full Ester | Pour Point in °C | Viscosity in cSt at 100° F | Viscosity in cSt at 210° F | Viscosity Index |
|------------|------------------|----------------------------|----------------------------|-----------------|
| A + 2D     | -60              | 28.03                      | 5.13                       | 124             |
| B + 3D     | -59              | 63.66                      | 8.86                       | 125             |
| C + 4D     | -54              | 88.15                      | 11.92                      | 136             |
| A + 2E     | -52              | 36.33                      | 6.29                       | 135             |

From the above Table III the extremely favorable properties for technical use of the ester oils according to the invention with reference to behavior to cold and of viscosity temperature behavior can be clearly noted. In spite of their relatively high viscosities and their favorable viscosity-temperature behavior (viscosity index), the products have an extremely low pour point of well below -30° C.

The previous specific embodiments are illustrative of the practice of the invention. It is to be understood, however, that other expedients known to those skilled in the art or disclosed herein may be employed without departing from the spirit of the invention or the scope of the appended claims.

15 We claim:

1. A branched-chain aliphatic ester oil consisting essentially of a full ester of a branched-chain aliphatic polyol having only from 2 to 6 primary hydroxyl groups selected from the group consisting of alkanepolyols having from 3 to 6 carbon atoms and alkoxylkanepolyols having from 6 to 12 carbon atoms with  $\alpha$ -branched-chain alcanoic acids having the formula



25 wherein  $\text{R}_1$  and  $\text{R}_2$  are straight-chained alkyl having from 1 to 19 carbon atoms and the total number of carbon atoms in the acid is from 14 to 22, said acids being selected from the group consisting of (1) acids derived from the oxidation of  $\alpha$ -branched alcohols formed from normal alcohols by the Guerbet synthesis and (2) an acid of the formula



35 40 2. The ester oil of claim 1 wherein said  $\alpha$ -branched alkanoic acid has 16 carbon atoms.

3. The ester oil of claim 2 wherein said  $\alpha$ -branched C<sub>16</sub>-alkanoic acid is an isopalmitic acid obtained by oxidation of the 2-hexyl-decanol formed from n-octanol by the Guerbet synthesis.

45 4. The ester oil of claim 1 wherein said polyol is a branched-chain alkanepolyol having only 2 to 4 primary hydroxyl groups.

5. The ester oil of claim 4 wherein said alkanepolyol is neopentylglycol.

50 6. The ester oil of claim 4 wherein said alkanepolyol is trimethylolpropane.

7. The ester oil of claim 5 wherein said alkanepolyol is pentaerythritol.

55 8. Lubricating and hydraulic fluid compositions containing from 20% to 100% by weight of at least one ester oil of claim 1.

9. In the process of facilitating the motion of one solid over the surface of another solid by providing a thin film of a lubricant between the surfaces of said solids in frictional contact, the improvement consisting essentially of utilizing at least one ester oil of claim 1 as said lubricant.

60 65 10. The ester oil of claim 1 being the triisopalmitic acid ester of trimethylolpropane, said isopalmitic acid being obtained by the oxidation of 2-hexyldecanol formed from n-octanol by the Guerbet synthesis.

\* \* \* \* \*